

## UNITED STATES PATENT OFFICE

2,215,244

## PROCESS OF MAKING PRESSED BOARD PRODUCTS

Harry K. Linzell, Greenville, Miss., assignor to  
United States Gypsum Company, Chicago, Ill.,  
a corporation of Illinois

No Drawing. Application July 3, 1935,  
Serial No. 29,733

4 Claims. (Cl. 92—55)

The present invention relates to a pressed board product and the process of its manufacture.

The primary object of the invention is the production of a hard, dense, coherent article of 5 synthetic lumber, usually in the form of boards or slabs which may be used for building purposes, interior decoration, panel boards, and the like.

One of the objects of the invention is the production of a board composed substantially of 10 cellulosic fibers or cellulosic and ligneous fibers in admixture with each other together with a comparatively small amount of a binder such as a hardenable oil in conjunction with auxiliary 15 binders formed as a result of partial pyrolytic decomposition of the cellulosic or ligneous fibers.

A further object of the invention is to produce 20 synthetic lumber by a process which involves the fibration of a ligneous substance such as wood, or various plants, either by a mechanical 25 or a chemical process, preferably the former, followed by the reassembly of the resulting fibers into a coherent mat or slab with the simultaneous incorporation with the fibers of a relatively small 30 amount of a hardenable oil. After the incorporation of the oil, the board may be subjected to heat and pressure within definite ranges, as will be more completely enumerated hereinbelow, whereby it will be consolidated into a hard, dense, coherent, water-resistant product.

The present process involves the formation 35 from the ligneous and cellulosic material of autogenously formed binders resulting from the pyrolytic decomposition of the ligneous material and its associated cellulosic complexes. The decomposition products then probably combine with 40 each other by condensation and polymerization, with the formation of resin-like binders which supplement the natural binders contained in the material. The presence of the oil further acts to bind the material closely together while at 45 the same time endowing it with properties of toughness and resilience.

The oils used may be of any suitable origin 50 and preferably comprise such oils as linseed oil, Perilla oil, China-wood or tung oil, soya bean oil, fish oils, menhaden oil, oil of Java olives, and other oils which have the property of hardening by drying, usually with the formation of what is 55 technically known as linoxyn. The size used upon the fibers may consist of the ordinary rosin size used in the form of a rosin soap, or may be a resin which is capable of saponification or emulsification, although it is understood that other water-proofing materials in the nature of

waxes such as paraffin wax, carnauba wax, cerasin wax, ozocerite wax, montan wax, and the like, may be used.

Broadly speaking, the present process comprises the fibration of ligneous material, although this does not exclude the use of fibers which have been chemically liberated from wood. Wood that has been merely mechanically fibrated forms the preferred embodiment of the invention. Assuming that the manufacture is to proceed on the basis 10 of the use of ground wood, which is usually ground in the presence of water by means of the usual pulp stones, the resulting pulp suspension is run into a suitable tank provided with an agitator and while therein is treated with, for example, rosin size in an amount approximately 1% to 2% of the weight of the fibers. At the same time there is run into the tank, preferably in the form of an emulsion, but not necessarily so, up to 10% of a hardenable oil as, for example, 15 linseed oil, Perilla oil, tung or China-wood oil, soya bean oil, fish oils, and the like. If thorough agitation is used, the previous emulsification of the oil is not absolutely essential, the main object being to obtain as thorough intermixing of the 20 oil, resin size and fibers as can reasonably be attained. After the oil and fibers have been mixed in the said tank, a sufficient quantity of a precipitant such as alum or aluminum sulfate is added 25 to decompose the rosin soap size, with the formation—in the usual manner—of an insoluble precipitate which deposits itself upon the fibers, at the same time carrying down with it the oil that has been added to the mixture. The result of 30 these treatments is that the resin now in the form of its aluminum complex and the oil are both deposited upon the fibers. The resultant suspension of sized and oiled fibers is now transferred to a suitable board-forming machine such as a Fourdrinier or Oliver board former, or other 35 mechanical equivalent device, upon which it is formed into a wet mat. This mat is then slightly compacted by being passed between squeeze rollers, all in the manner well known in this art, whereupon the resultant damp mats are transferred to a drier wherein they are dried at a 40 temperature above 212° F., with the removal of all or substantially all of the moisture therein contained. During this drying there takes place a hardening of the oil, with the formation of 45 linoxyn. As the time of hardening and formation of linoxyn varies with the type of oil used, it may be advisable to store the dry boards for from a day or so to a few weeks, depending upon the 50 rate at which the various oils which may be em- 55

ployed oxidize. It has been found that excellent results are obtained when the oil is dried to the state where it becomes merely plastic when subjected to heat and pressure. In order to enhance 5 the hardening of the oil, it will, of course, be possible to add to the oil a small amount of the well known driers such as manganese, cobalt, or lead compounds, which are known in the paint and varnish industry; and in claiming oils herein 10 it is to be understood that these may include such driers. In place of the rosin size, or conjointly therewith, there may also be used a small percentage, say 2%, of the aforementioned paraffin or waxes, these being incorporated preferably in 15 either finely divided or emulsified form, although their use in the form of saponification products or soaps is not to be excluded.

Assuming for the purposes of the present description that a board having two plane flat surfaces is to be made, the board is first thoroughly relieved of all the therein contained vaporizable matter or moisture, and the board is then placed between heated surfaces, such for example as the platens of a hydraulic press, whereupon impacting pressure is applied to said boards of from 20 500 to 3000 pounds per square inch for a period of from one minute up to one hour at a temperature range of from 350° F. upward, but short of the point of active development of carbon for the 25 materials. The ignition point of wood is about 30 527° F. As a result of the applied pressure there is brought about a consolidation of the board while at the same time the heat tends to decompose the cellulosic and ligneous constituents 35 thereof, with the autogenous formation of resinous and tarry condensation products which act as auxiliary binders and serve to bind the fibers of the board together into a strong and coherent mass. The function of the oil and water- 40 proofing agents is greatly to enhance the resistance of the product to the inter-penetration of liquids such as water, thus producing a dense water-repellent and water-resistant board.

If, on the contrary, the mats have been stored 45 for some time in order to permit hardening of the oils, the boards will then contain hygroscopic moisture which they have picked up from the atmosphere. Boards containing such moisture can be pressed if there be interposed between 50 at least one surface thereof and the heated platens some foraminous material such as a screen, in order to permit the escape of moisture which is converted into steam because of the heat imparted to the mats by their contact with 55 the surfaces of the platens.

In order to prevent possible difficulties resulting from the adhesion of the boards to the platens of the press, it is preferable to interpose between the boards and the platens heat-conducting caulk plates of oxidized metal or sheets coated with enamel or a glass-like composition. In stating the temperatures used in the present process, it is understood that these temperatures are measured at the surface of the metallic heat-conducting bodies that are in contact with the boards. Of course, if the platens themselves are of oxidized metal or are coated with enamel or other glass-like composition, such intermediate sheets may then be dispensed with. At any rate, 60 the temperatures mentioned are the temperatures in contact with the board and not the temperatures of the interior of the platens themselves.

As a specific embodiment of the present invention, it may be stated that if a board sized with

rosin and containing a hardenable oil is to be pressed, the temperature is preferably above 350° but below the point of active carbon formation.

Instead of forming the board wet, it is possible to proceed by first producing dry fibrated wood, 5 as by grinding the same. The thus produced fibers are then mechanically mixed with a small amount of the above-mentioned oily substances to form fibers having these substances adhering thereto. The thus treated fibers are then stored, 10 either hot or cold, to allow the added oil to harden. Thereupon the fibers are mechanically made into a mat, as by blowing them with an air current onto a foraminous surface while applying suction to the latter. This mat is then 15 laid onto the platens or the oxidized or enamelled caulk plates, and pressed in the manner already described.

The pressing time depends, of course, upon the temperature and the pressure used. It may be 20 stated, as a general rule, that as the temperature increases the time may safely be decreased, so that near the upper end of the temperature range stated the pressing time may be a matter of but a few minutes while at the lower end it 25 may extend from one-half to one hour.

A somewhat similar effect is noticed in the case of pressures, and as a general rule the higher the pressure the shorter may be the pressing time, in order to secure a board of approximately 30 the same density, although it is not to be understood that the relationship of the pressure to the time is the same as that of the temperature to the time. Thus, if both a high pressure and a high 35 temperature are used, the resultant product will be very hard and very dense and may be pressed in a comparatively short time, whilst on the contrary, if the pressure is light and the temperature is low, the pressing time must be correspondingly lengthened, but in the latter case the density will 40 be lower.

When pressing a board, a temperature between 425° F. and 475° F. is suitable.

One of the advantages in interposing an oxidized metal caulk plate or an enamelled or glass-lined caulk plate between the boards being pressed and the platens is that such plates require little or no greasing or oiling, as they are naturally endowed with a tendency to obviate the sticking of the boards. This greatly simplifies manipulation and greatly facilitates rapid and economical manufacturing operations.

In carrying the present invention into commercial practice, it has been found that there are distinct advantages in applying the impacting pressures in distinct stages or intervals, the pressure being either the same at each period or different in each of the periods, as will presently be explained. In any event, there is a release of pressure between the individual impactions. For 60 example, sheets of insulating board completely relieved of their moisture, are placed on caulk plates and the assembly inserted between the platens of a hydraulic press. The temperature as measured at the surface of these platens may be, for example, between 450° F. and 455° F. The press is then operated so as to bring the platens into contact with the boards, but without the application of any substantial pressure, for the purpose of heating the surface of the boards to about the 65 temperature of the platens. This usually takes from one to three minutes. During this time, which can conveniently be termed the "toasting period," the board surface will have acquired a 70 temperature sufficiently high so as to prevent the 75

adhesion of the boards to the caul plates. The pressure is then applied for a period of from two to three minutes, whereupon it is gradually released and the platens allowed to lift slightly off the boards for the purpose of allowing the escape of the accumulated gases and vapors. A bluish acrid smoke will be seen to rise from the boards and pass out between the platens. The pressure is then again applied for a further period of from two to three minutes, whereupon it is again released in the same manner as already described. The pressure is then once more applied, and at the end of another period of two or three minutes the pressure is finally released and the press opened. Thereupon the boards are quickly removed from the press and immediately subjected to a strong blast of air, preferably but not necessarily heated, to remove as much as possible of the smoke and gases from the freshly formed boards. This is done in order to remove the somewhat acrid odor which would otherwise adhere to the boards. The boards may then be passed through a passageway in which they are subjected to a blast or current of cool air in order to relieve them of heat and allow them to assume room temperature without warping.

It has been found particularly advantageous to change the pressure during the various times that it is applied, this pressure either increasing or, in some instances, being lowered. For example, when making a hardened board  $\frac{1}{8}$  inch thick and of a density of from 65 to 75 pounds per cubic foot and working at a temperature of 450° to 455° F., measured at the surface of the platens, the cycle may be substantially as follows: The board is subjected to the toasting operation at a pressure of not exceeding 50 pounds for a period of one minute, whereupon the pressure is released momentarily to allow the escape of the initial amount of smoke and gases formed. The pressure on the boards is then raised to 400 pounds per square inch for a period of two minutes, whereupon it is released and the platens lifted clear of the boards. The pressure is then applied to the extent of 800 pounds per square inch and kept on for a period of two and one-half minutes, whereupon it is again released and the platens lifted from the board. There then follows a final application of pressure on the order of 1200 pounds per square inch for a period of three minutes, at the end of which time the pressure is released, the press opened and the boards removed. The total pressing time counting from the moment the boards enter the press, and therefore including the toasting period of one minute, is thus eight and one-half minutes.

As an example of the production of  $\frac{3}{16}$  inch hard board at 450° to 455° F. and having a density of 65 to 70 per cubic foot, it may be stated that the entire cycle is somewhat longer, namely, about ten and one-half minutes, because of the fact that  $\frac{3}{16}$  inch board is 50% thicker than  $\frac{1}{8}$  inch board and that therefore the mass of material is 150% of that of the  $\frac{1}{8}$  inch board. Inasmuch as the heat is abstracted from the surface of the board by the loose-textured interior, it takes a little longer to get the surface of the board up to the platen temperatures, which makes it necessary slightly to increase the toasting period in this case 50%. Thus, in making the  $\frac{3}{16}$  inch board, three intermediate pressure releases and the final pressure release, and three stages of pressure application respectively of 400, 800 and 1200 pounds per

square inch, these periods being 3, 3 and 3½ minutes respectively, are employed. The total time, counting from the moment that the board enters the press and including the 1½ minute toasting period at less than 50 pounds pressure, is therefore 10½ minutes.

In the manufacture of  $\frac{1}{4}$  inch hard board at 450° to 455° F., the cycle is somewhat different. The toasting period in this case at less than 50 pounds pressure is 2 minutes. The first application of pressure for a period of 2½ minutes is 400 pounds, followed by two separate applications of pressure of 3 minutes each at 800 pounds, and finally application of 1200 pounds pressure for 3½ minutes, or a total of 14 minutes, counting from the time the board enters the press.

Alternatively, in making  $\frac{1}{8}$  inch hard board of a density of 65 to 70 pounds per cubic foot, at 450° to 455° F., the applications of pressure may all be of the same degree, viz., 1000 pounds. Thus the initial toasting period may be one minute, followed by release of pressure and lifting of the platens from the boards, whereupon pressure of 1000 pounds is applied for 1½ minutes, followed by pressure release and lifting of the platens just as previously described. The pressure is then again raised to 1000 pounds for 2 minutes, again released and then once more raised to 1000 pounds per square inch for a period of 2½ minutes, whereupon the pressure is released and the press is opened. The total time, therefore, including the toasting period, is 7 minutes. When operating in this manner, however, the results are not as completely satisfactory as they are when working in accordance with the conditions where there are increments in pressure, for it appears that the development of the smoke and gases tends to the formation of a fiber board which shows a slight inclination toward blistering or laminating and also has a greater tendency to stick to the caul plates than when the pressure is applied in increments. It will be noticed, however, that the cycle is 1½ minutes shorter and the highest pressure is 200 pounds less, that is, 1000 pounds instead of 1200 pounds.

Still another way of operating, when making  $\frac{1}{8}$  inch board at 450° to 455° F. and of a density of 65 to 70 pounds per cubic foot, is as follows: When working in accordance with the following conditions, the tendency of the board to laminate is very slight. In this type of cycle there is the usual toasting period of 1½ minutes with a pressure of less than 50 pounds, followed by a pressure release and lifting of the platens from the board, whereupon a higher pressure of 1500 pounds per square inch is applied for a period of 1½ minutes. The pressure is then released and the platens merely placed in contact with the boards, just as during the toasting period, and held that way for 4 minutes at a pressure of less than 50 pounds. During this prolonged second toasting period an opportunity is given for full development of the desired quota of resinous and tarry materials as a result of the pyrolytic decomposition of the wood. The pressure is then released to allow gases and smoke to escape by lifting the platens from the board, whereupon the pressure is again applied to the full 1500 pounds for a period of 3 minutes. During this latter period the resins formed during the 4-minute toasting period, together with such additional resins as form during the second compression stage, are set and the board is given its final hardness. The total pressing time, including the initial toasting, is thus 10 minutes.

When working in this manner, but raising the temperature say from 462° to 464° F., the total time cycle could easily be reduced to 7 minutes by shortening the intermediate toasting stage as well as the compression stages, as will be readily understood from what has been said above.

It is also possible, although not as advantageous, to work at a lower temperature such as 400° F., but in that case the time cycle is very greatly increased. This increase in time cycle, however, is compensated for by other advantages, viz., that less pressure need be carried on the boiler that furnishes the high pressure steam for heating the platens and also that the skill of the press-operator need not be of as high order, nor need the cycles be so slavishly adhered to. In other words, when working at the lower end of the temperature range, and producing a  $\frac{1}{8}$  inch hard board, a temperature of 400° might be used. In that case the initial toasting is 5 minutes. There is an application of pressure of 500 pounds for 9 minutes, two applications of 1000 pounds for 10 and 11 minutes, respectively, and two applications of 1500 pounds for 12 and 13 minutes, respectively, making a total time, including the toasting, of 60 minutes. It will be obvious that at 400° F. these intermediate cycles may be shifted about as to time without seriously interfering with the successful operation of the process. Furthermore, a variation in the total time of 10% in either direction would make very little difference. Where a 20-stage press, for example, is used and there is but one operator, it is quite possible that the same operator could thus handle two presses, making twenty boards at a time, having time to attend to both of them without interfering with the proper carrying out of his duties.

The manufacture of what may be called a semi-hard board, having a density of from 39 to 50 pounds per cubic foot, which is made by using stops to prevent the travel of the platens beyond the limits thereof, is about as follows: The stops are  $\frac{1}{4}$  inch thick, so that the board will under no circumstances be thinner than  $\frac{1}{4}$  inch. The pressing cycle is somewhat different. The initial toasting period is one minute. There is then an application of pressure of 250 pounds for 2 minutes, followed by the usual pressure release, followed by a cycle of 500 pounds pressure for 3 minutes, which suffices to compress the board up to the limits of the stops, whereupon the pressure is released and the platens lifted as usual. The final application of pressure need therefore be only 250 pounds, because there would be no object in applying any greater pressure than would be necessary to bring the re-expansion of the board above the limits of the stops. The total cycle in that particular example is  $9\frac{1}{2}$  minutes. Obviously, the initial toasting may be carried out under the full pressure of the press.

The boards produced by the present process have a high modulus of rupture, have low water absorption and a pleasing and smooth polished surface. The fibers therein are consolidated together and coalesced by the production of autogenously produced resins and tarry condensation products which result from the heating of the therein contained cellulosic complexes, lignins, and the like. The inherent water-resistance and bonding powers of these autogenously produced binders is further enhanced by the simultaneous presence of the hardened oils and the rosin size, which tends to plasticize the autogenously pro-

duced binders. It will be noted that the amount of rosin size and oils is relatively small, and unless the temperatures were within the range given, these oils would by themselves be insufficient to produce a board having the same degree of strength and water resistance. It is, therefore, the cooperation of the autogenously formed binders with the added oils which mutually contributes to the high degree of water resistance, lack of water absorption and final strength of the products made in accordance with the present invention.

Applicant is aware of the fact that waxes, oils and sizes have been used in the past for the purpose of enhancing the water resistance of fibrous products, but he is not aware that the autogenous development of resins and condensation products conjointly with the use of hardened oils has ever been used before and therefore considers this as a distinct step in advance and as forming one of the essential elements of his present invention, for which he claims:

1. The process of forming a hard, dense, consolidated product consisting essentially of cellulosic and ligneous fibers in an interlaced condition, which comprises precipitating upon said fibers a metallic resinate and a drying oil while said fibers are suspended in a liquid, separating said fibers from said liquid to form a coherent wet mat, removing the water from said mat and effecting the drying of said oil by oxidizing it, further drying the resultant product until all free moisture is removed therefrom, and thereupon compacting the resultant coherent mat by means of heat-conducting surfaces maintained at from 350° F. to below the point of carbon development under an intermittently applied pressure of from 400 to 3000 pounds per square inch for a time sufficient to effect substantial thermolysis of the therein contained ligneous and cellulosic fibers.

2. The process of consolidating ligneous cellulosic material into a dense, compact, coherent board or slab which comprises the steps of mixing such material with a drying oil, forming the material into a coherent but pervious mat, removing the moisture from said mat and oxidizing the drying oil to a sufficient extent to cause it to become dry, and thereafter pressing the resultant mat at a pressure of from 500 to 3000 pounds per square inch at a temperature of at least 350° F. but short of a temperature high enough to cause development of carbon.

3. The process of consolidating ligneous cellulosic material into a dense, compact, coherent board or slab which comprises the steps of mixing said material with waterproofing material and a drying oil, forming the resultant mixture into a coherent but pervious mat, removing the moisture from said mat and subjecting the same to oxidizing conditions for a time sufficient to effect the oxidation of said drying oil so as to cause it to become dry and thereafter pressing the resultant mat at a temperature of at least 350° F. but short of a temperature high enough to cause development of carbon.

4. The process of forming a hard, dense, consolidated lignocellulosic product which comprises fibrating lignocellulosic material so as to yield a mixture of cellulosic and ligneous fibers, precipitating upon said fibers a waterproofing material and a drying oil, forming the thus treated fibers into a coherent mat, subjecting said mat to drying and oxidizing conditions so as to remove the

moisture therefrom and to oxidize said drying oil so that the same becomes dry, and thereupon subjecting the resultant product to intermittently applied compacting pressure while confined between metallic heat-conducting surfaces, which latter are at a surface temperature of at least

350° F. but short of a temperature high enough to cause development of carbon for a length of time sufficient to produce autogenously formed resinous binders as a result of the ensuing thermolysis of the same.

5

HARRY K. LINZELL.